

# UNITED STATES PATENT OFFICE.

ALBERTO DE SALAS, OF MEXICO, MEXICO.

## PROCESS OF PREPARING FLOCK-COTTON FOR EXPLOSIVES.

1,249,726.

Specification of Letters Patent. Patented Dec. 11, 1917.

No Drawing.

Application filed July 19, 1917. Serial No. 181,590.

To all whom it may concern:

Be it known that I ALBERTO DE SALAS, a subject of Spain, and a resident of the city of Mexico, country of Mexico, have invented certain new and useful Improvements in Processes of Preparing Flock-Cotton for Explosives, of which the following is a specification.

The object of this invention is to provide 10 a means of recovering from such materials as soiled cotton rags, machinists' waste, garment manufacturers' cuttings, and discarded clothing, a suitable and inexpensive substitute for the raw or bloom cotton heretofore 15 used in the manufacture of smokeless powder, guncotton, and other varieties of explosives in which nitrated cotton is an important ingredient.

For the preparation of flock cotton from 20 new or fairly clean rags, a tank with a solution of sodium soap is provided, one hundred kilos of rags requiring five hundred liters of water and from three to five kilos of the soap. The soap is dissolved by boiling 25 from four to five hours, preferably in small containers. After the solution has become tepid, one kilo of bicarbonate of soda is added and the rags are soaked in the cold solution for about eight hours. They are 30 then wrung out and washed either in clean running water or clean water which is changed at intervals of two hours until no further impurities are washed out. The rags are then wrung out and dried in the 35 sun and picked apart into a flocculent condition either by hand or by passing through a teaseling machine. This is followed if necessary with a second treatment which may be with a solution of the same composition and for the same length of time, but 40 which is preferably a soap solution prepared as before but to which about five grams of anilin oil is added while tepid. Then after wringing out, the rags are again washed 45 either in clean running water or clean water which is changed about every six hours until the rags are thoroughly clean. Then after wringing out and drying in the sun they are again brought into a flocculent condition 50 either by raveling by hand or by passing through a teaseling machine.

For the preparation of flock cotton from rags which are dirty or contain grease, the treatment may be substantially the same except for an increase in the strength of the 55 solution as to some or all of the ingredients

according to the amount of dirt and grease to be removed. In the case of very dirty and greasy rags a suitable solution for the first treatment consists of five hundred 60 liters of water in which eight kilos of sodium soap have been dissolved by boiling, five kilos of bicarbonate of soda added while the solution is hot, and about ten grams of anilin oil. The rags are soaked for eight hours in 65 the cold solution, then wrung out, and washed in frequently changed or running water until no further impurities are washed out. They are then wrung out, dried in the sun and brought into a flocculent condition. 70 This is followed by washing with water in which one or two per cent. of soap has been dissolved by boiling. A second treatment is then given in which the wrung-out material is put into a tank containing a new 75 solution and soaked for about twelve hours. This solution consists of one thousand liters of water, ten kilos of normal carbonate of soda and fifteen kilos of ammonia. It is kept at a temperature of 50° C., and the 80 flock is kept stirred under for twelve hours. Then it is wrung out and washed in frequently changed clean tepid water for six 85 hours and the washing continued in clean running water until it loses its odor. Then it is wrung out and after being dried in the sun is brought into a flocculent condition by passing three times through a teaseling machine.

The foregoing detailed description has 90 been given for clearness of understanding and no undue limitation should be deduced therefrom, but the appended claims should be construed as broadly as permissible in view of the prior art.

What I claim as new and desire to secure by Letters Patent of the United States is:

1. The process of preparing flock cotton which consists in soaking rags in a solution of soap and an alkali, washing, drying, and 100 mechanically bringing into a flocculent condition, substantially as described and for the purpose set forth.

2. The process of preparing flock cotton, which consists in soaking rags in a solution 105 of sodium soap and bicarbonate of soda, washing, drying and mechanically bringing into a flocculent condition, substantially as described and for the purpose set forth.

3. The process of preparing flock cotton, 110 which consists in soaking rags in a solution of sodium soap, bicarbonate of soda, and

anilin oil, washing, drying, and mechanically bringing into a flocculent condition, substantially as described and for the purpose set forth.

- 5 4. The process of preparing flock cotton, which consists in soaking rags in a solution of sodium soap, bicarbonate of soda, and anilin oil, washing, drying, and mechanically bringing into a flocculent condition
- 10 and retreating with a solution of normal

carbonate of soda and ammonia, substantially as described and for the purpose set forth.

Signed at New York, N. Y., this 16th day of July, 1917.

ALBERTO DE SALAS.

Witnesses:

SAMUEL W. BALCH,

PEDRO REQUENA-LEGARRETA.